

## UNITED STATES PATENT OFFICE

JAMES A. PARSONS, JR., OF DAYTON, OHIO, ASSIGNOR TO THE DURIRON COMPANY, INC., A CORPORATION OF NEW YORK

## IRON ALLOY

No Drawing.

Application filed January 10, 1929. Serial No. 331,708.

The invention relates to iron alloys, and is in part a continuation of my application, Serial No. 240,929. It has for its objects the provision of an improved alloy of the iron 5 silicon class, having high acid resisting qualities, which is tougher and more resistant to impact than those heretofore produced, which gives a denser casting, free from gas inclusion or voids, and which, in general, has 10 a wider field of service and greater reliability than alloys of this class heretofore developed.

I have found that alloys of iron and silicon, in which the silicon content ranges from 15 9 to 20 per cent, and which are relatively weak and brittle and subject to fracture on impact and sudden change in temperature, may be greatly improved by the use of certain of the carbide forming metals in connection with 20 carbon and by the use of nickel or cobalt. By the use of these elements properly proportioned, I have found that strength of the alloy may be doubled and its acid resisting qualities increased five or six times. The use 25 of the carbide forming metals in conjunction with the carbon provides the necessary amount of combined carbon to give the alloy its high corrosion resisting quality. Without such elements, when sand castings are 30 made from high silicon iron alloys, all the carbon in the casting is in the form of graphite, and there is present substantially no combined carbon. Further, such graphite is in the form of flakes. By the addition of cobalt 35 or nickel, the flakes are changed to nodules, which results in a large increase in the tensile strength of the casting. The amount of nickel or cobalt added must, however, be limited for two reasons. First, nickel in amounts 40 over 1.5 per cent materially reduces the acid resisting properties of the alloy, regardless of the silicon or carbon content. Second, the nickel or cobalt acts in the alloy to precipitate the carbon as graphite, so that it is not 45 desirable to introduce more of these elements than is necessary to change the graphite from the flake to the nodule form, otherwise, the effect incident to the addition of the carbide forming metals will be defeated, as there will 50 not be sufficient carbon left unprecipitated in

the alloy to combine with the carbide forming metals.

The carbide forming metals, which I have found suitable to add to the alloy are tungsten, vanadium and molybdenum, the elements being stated in the order of their affinity for carbon, the tungsten and vanadium being more suitable for this reason than the molybdenum. It will be understood that the three elements may be used in the alloy individually or in combination. The nickel and cobalt may similarly be used in the alloy together or separately. The following is a specific example of proportions and elements giving the improved alloy:

|                                                        | Per cent |
|--------------------------------------------------------|----------|
| Silicon                                                | 14       |
| Nickel or cobalt or combinations thereof               | 1        |
| Tungsten, vanadium, molybdenum or combinations thereof | 2        |
| Carbon                                                 | 0.8      |
| Iron                                                   | Balance  |

However, the proportion may vary over a considerable range, while still retaining in the alloy in a large degree the improved characteristics as above set forth. These proportions may vary in accordance with the following limits:

|                                                        | Per cent   |
|--------------------------------------------------------|------------|
| Silicon                                                | 9 to 20    |
| Nickel or cobalt or combinations thereof               | 0.1 to 3   |
| Tungsten, vanadium, molybdenum or combinations thereof | 0.1 to 10  |
| Carbon                                                 | 0.1 to 1.5 |
| Iron                                                   | Balance    |

It will also be understood that the invention comprehends the use of other elements in the alloys, in such relatively small quantities as will not materially affect the character 90 of the alloys. Small amounts of sulphur, phosphorus, manganese and the like, which occur more or less as impurities, will also be understood to be comprehended by this invention.

What I claim is:

1. An iron silicon alloy consisting of from 9 to 20 per cent of silicon, from 1 to 3 per cent of nickel, 0.1 to 10 per cent of metal belonging to the group tungsten, vanadium and 100

molybdenum, sufficient carbon to combine with such metal and the balance iron.

2. An iron silicon alloy consisting of from 9 to 20 per cent of silicon, from 1 to 3 per cent of nickel, 0.1 to 10 per cent of metal belonging to the group tungsten, vanadium and molybdenum, from 0.1 to 1.5 per cent of carbon, and the balance iron.

3. An iron silicon alloy consisting of from 10 9 to 20 per cent of silicon, from 1 to 3 per cent of metal belonging to the group nickel and cobalt, 0.1 to 10 per cent of metal belonging to the group tungsten, vanadium and molybdenum, sufficient carbon to combine with such 15 last metal and the balance iron.

4. An iron silicon alloy consisting of about 14 per cent silicon, about 1 per cent of metal belonging to the group nickel and cobalt, about 2 per cent of metal belonging to the 20 group tungsten, vanadium and molybdenum, about 0.8 per cent carbon and the balance iron.

In testimony whereof, I have hereunto subscribed my name this 8th day of January, 1929.

25

JAMES A. PARSONS, JR.

30

35

40

45

50

55

60

65